

## UNITED STATES PATENT OFFICE

1,970,067

## PROCESS FOR THE PRODUCTION OF AGE-RESISTING IRON AND STEEL

Carl Wallmann, Fritz Halbrock, and Emil Kumpmann, Mulheim-on-the-Ruhr, Germany

No Drawing. Application June 30, 1932, Serial No. 620,309. In Germany January 22, 1932

1 Claim. (Cl. 75—27)

This invention relates to a process for the production of age-resisting iron and steel.

It is known to produce age-resisting iron or steel, that is to say, iron or steel which, on aging, do not exhibit any substantially increased brittleness in suitable test pieces. Up to the present, it has been possible to produce such iron and steel in different ways. The age-resisting property is obtained, for example, by treating the iron or steel with desoxidizing agents, during the melting and the maintenance of definite conditions, to a larger extent than is otherwise customary in melting ordinary kinds of iron and steel. Another way of obtaining the age-resisting property consists of a normalizing heat treatment (quenching and annealing) and also in hot working at temperatures in the vicinity of the upper transformation point. Finally, the age-resisting property can also be imparted by alloying 20 with certain metals, such as chromium, nickel, copper and the like.

All these processes increase, to a certain extent, the cost of the articles that are to be manufactured from age-resisting iron or steel, because 25 they all entail operations additional to the ordinary manufacturing operations, thereby naturally increasing the cost of the finished products. This is particularly the case when the age-resisting property is obtained by alloying, special 30 heat treatment, and shaping within special ranges of temperatures.

Moreover, when known desoxidizing agents, such as aluminium, are employed, inclusions (in that case, of alumina) may be formed, which 35 remain in the iron and steel and may cause, on their surfaces of fracture, defective places which render the employment of the piece questionable. As a rule, the desoxidizing agent employed for the production of age-resisting steels by extensive desoxidation, is added in the furnace, shortly before tapping, or else, after tapping, in the 40 ladle. For this reason, in many instances, only a very short time is available for the desoxidation and it then easily happens that the intended age-45 resisting property of the steel is not obtained, this result being equivalent to a wasted charge.

Another defect arising in the production of age-resisting kinds of iron and steel, and also those in which that property is not required, is 50 the circumstance that the slag of the molten bath,

whilst taking up, in the desired manner, undesirable constituents of the bath (principally sulphur and phosphorus), also takes up constituents which are desired to remain in the iron and steel that is being produced.

In the usual melting process, it is customary, for absorbing sulphur and phosphorus from the bath, to add an abundant quantity of lime after the charge has melted down, a basic slag possessing the desired capacity for absorbing sulphur 55 and phosphorus, being thereby formed.

Among the constituents which pass, contrary to desire, into this basic slag, is (inter alia) the manganese in the charge. In the most usual manner of conducting the melting process, it is 60 the practice to replace the manganese which has passed into the slag, and therefore become lost to the bath, by adding fresh manganese (in the form of ferro-manganese) to the bath towards the end of the process compensating for that manganese which has gone into the slag, thereby becoming useless for the bath, in order to obtain the 65 desired end product.

However, as with the aforesaid addition of desoxidizing agents, such as aluminium, the addition of ferro-manganese towards the end of the 70 melting process, gives rise to defects in the form of inclusions of manganese sulphide and manganese silicate—derived from the ferro-manganese—which inclusions may remain in the solidifying iron or steel, and impair its usefulness. In 75 addition to the aforesaid inconveniences, the addition of ferro-manganese towards the end of the melting process, in the manner now generally employed in the melting operation in the Siemens-Martin process, considerably increases the 80 cost of the product.

On this account, attempts have been made to 85 recover the manganese from the slag by the addition of welding slag and iron ore—or in some cases, only one of these agents—to the molten charge.

Said processes are, however, accompanied by several drawbacks. The addition of iron ore or 90 welding slag introduces additional oxygen into the bath, and experience shows that the removal of this oxygen is necessary and desirable. Moreover, it is doubtful whether, in adding lime after the ore and at a time when the temperature of the bath is very high, the part ascribed to the 95 molten bath,

lime of absorbing sulphur and phosphorus from the bath, can be adequately performed.

Generally, in all these processes, viscous slags are produced, the rapidity of the reaction intended to take place between the slag and the bath being thereby unfavourably affected. It is therefore necessary, in many cases, to add fluor-spar to these viscous slags, in order to improve their fluidity and thus assure the desired rapidity 10 of the reaction.

The difficulties occurring in the above processes are excluded by the process according to the present invention, and the advantages aimed at in the aforesaid known process—such as reduction 15 of cost by lowering the addition of ferro-manganese, and obtaining age-resisting iron or steel without the excessive employment of desoxidizing agents liable to lead to inclusions—are assured in a manner that is easily carried out in practice.

20 In the process of the present invention the early stage is carried through in the usual known manner. As is customary in the pig and scrap or iron ore process, the charge is proportioned, so as to bear in mind the desired end figures for 25 manganese, carbon and so forth, and is mixed with a sufficient amount of lime to meet the requirements of the entire process. The whole can then be melted down, in any ordinary Siemens-Martin furnace, in the usual way, the abundant 30 addition of lime forming a basic Martin slag. The abundant proportion of lime in the charge is able to exert a favourable action, especially at the low temperature of the first stage of the melting process, inasmuch as a more and extensive refining, in respect of sulphur and phosphorus, is 35 thereby effected than if the lime were introduced at a later stage of the process.

When the melting process has sufficiently progressed for the lime—usually employed in lump 40 form—to have risen to the surface, silica, in the form of sand, refractory material, glass, or the like, is added in a larger amount than hitherto customary, in fact, sufficient to acidify the originally basic slag, and to form a slag with a concentration ratio of silica to lime that is best adapted to prevent migration of the manganese from the bath into the slag, and to reduce such manganese as has already passed into the slag, without permitting any detectable return of sulphur 45 and phosphorus from the slag into the bath. Investigations have proved this ratio to be best adapted at from 1 to 1.5 up to 1 to 2. By the process of the present invention therefore, subsequent additions of ferro-manganese are obviated, and the usual addition of ore, with its—in 50 any event—undesirable introduction of oxygen, is rendered superfluous.

A further effect of the acidification of the, originally basic, slag by a copious addition of sand 60 or the like, is to be seen in the decomposition of compounds of iron and oxygen in the slag and the resulting decrease in the iron content of the latter. This is equivalent to an increased yield of steel, in this process, as compared with that furnished by the existing processes for producing steel in ordinary Siemens-Martin furnaces.

Since the absorption of manganese by the slag is prevented in all the operations according to the 70 present process, the latter also precludes the risk of inclusions—in the form of manganese sulphides or silicates—in the finished steel. It also excludes the risk of alumina inclusions, by dispensing with the addition of aluminium. The injurious 75 effect of such inclusions on the physical prop-

erties of the steel is sufficiently well known, and emphasises the advantages afforded by the present process.

A further advantage of the present process consists in that the increased fluidity of the slag through the addition of large amounts of sand, or the like, allows all the reactions between the bath and the slag to proceed with the desired speed, so that there is no need for the addition of fluor spar, or similar material, which would increase the cost.

80 The following examples represent: (A) the process according to the present invention; and (B) a current process. In both cases, the charges 85 are intended to produce plate material.

#### Example A

|                                                                                 | Charge     |     |
|---------------------------------------------------------------------------------|------------|-----|
| Pig-iron.....                                                                   | 22000 kgs. | 95  |
| Tube scrap.....                                                                 | 16900 "    |     |
| Crop ends.....                                                                  | 12500 "    |     |
| Strip scrap.....                                                                | 3500 "     |     |
| Turnings.....                                                                   | 7000 "     |     |
| Bay scrap, waste material which is produced at the casting of steel blooms..... | 5000 "     | 100 |
| Caucasian washed manganese ore (52%).....                                       | 500 "      |     |
| Ferrosilicon (78%).....                                                         | 300 "      |     |
| Total charge.....                                                               | 67700 "    | 105 |
| Yield.....                                                                      | 64360 "    |     |

Analysis: 0.22% C, 0.72% Mn, 0.21% Si, 0.031% P, 0.031% S.

110 The run took 9 hours, and 3000 kgs. of lime were added, and melted down, with the charge, this stage occupying 7 hours 25 minutes. 900 kgs. of sand were required for the recovery of the manganese. The melting proceeded satisfactorily, but no addition of iron ore was given, which accounts for the greater length of the run. No desoxidizing agents were employed.

#### Example B

|                              | Charge     |     |
|------------------------------|------------|-----|
| Pig-iron.....                | 15000 kgs. |     |
| Heavy melting scrap.....     | 16900 "    |     |
| Strip scrap.....             | 6900 "     |     |
| Plate sides and ends.....    | 23100 "    | 125 |
| Tube scrap.....              | 5000 "     |     |
|                              | 66900 "    |     |
| Ferro-manganese (80%).....   | 800 "      |     |
| Ferro-silicon-aluminium..... | 260 "      | 130 |
| Total.....                   | 67960 "    |     |
| Yield.....                   | 64860 "    |     |

Analysis: 0.19% C, 0.53% Mn, 0.14% Si, 0.015% P, 0.037% S.

135 The run took 7 hours 35 minutes. 3000 kgs. of lime were melted down with the charge, and about 1000 kgs. of lime and 500 kgs. of fluor spar were added later. The melt was desoxidized with ferro-manganese or ferro-silicon-aluminium.

The examples speak for themselves.

As is to be seen from Example A the slag is acidified to such a degree that the basicity of the 145 slag is substantially decreased whereas it is not intended to transfer the original basic slag into an acid one. It will thus be understood that by "acidifying" referred to in the specification and in the claim it is only intended to characterize a 150

process by which the basicity of the slag is substantially diminished without however transferring it into the acidic character.

We claim:—

5 A process for the production of age resisting iron and steel in a basic open hearth furnace comprising charging the furnace with a melting charge consisting of crude iron scrap and lime, melting said charge down until it has become fluid

and the lime is floating upon the surface, acidifying the basic slag thus formed and transferring the slagged manganese from the slag into the bath and finally tapping the melt after it has obtained the desired properties.

80

10

85

15

90

20

95

25

100

30

105

35

110

40

115

45

120

50

125

55

130

60

135

65

140

70

145

75

150

CARL WALLMANN.  
FRITZ HALBROCK.  
EMIL KUMPMANN.